

## UNITED STATES PATENT OFFICE

2,522,512

## PREPARATION OF SYNTHETIC LUBRICANT

Denham Harman and William E. Vaughan,  
Berkeley, Calif., assignors to Shell Development  
Company, San Francisco, Calif., a corporation  
of Delaware

No Drawing. Application October 5, 1946,  
Serial No. 701,412

10 Claims. (Cl. 260—609)

1

This invention relates to novel lubricating compositions. More particularly, it pertains to the use of certain fractions of non-mineral oil base sulfur-containing compounds, especially for low temperature and/or extreme pressure lubrication.

The use of mineral oil fractions for lubricating is suitable for many purposes, but it is well-known that such lubricants possess certain inherent limitations, such as tendency to oxidize, thickening at low temperatures, etc. A large number of additives have been employed with mineral oils in order to improve these shortcomings. To a certain degree, the resulting compositions may be used successfully for most lubricating purposes.

Various synthetic lubricants have been proposed from time to time. These include polymers of cracked wax olefins, alkylated aromatics and so on. Some of these are useful for special purposes, but, especially if the previously known synthetic lubricants were derived from olefinic sources, they usually possessed corrosion and oxidation characteristics limiting their utility to a substantial degree. Another type of synthetic lubricant which has been investigated is the alkylene oxide polymer type, such as polymerized propylene oxide.

The preparation of adducts of certain unsaturated compounds with hydrogen sulfide or mercaptans has also been proposed. However, especially when reacting hydrogen sulfide with di-olefins, a complicated mixture of derivatives is present in these adduct products. The mixtures prepared by previously proposed methods contain relatively large proportions of volatile constituents as defined hereinafter, with a correspondingly lower proportion having lubricating properties, dependent upon the identity and quantity of catalyst employed.

It is an object of the present invention to provide a novel method for the production of a non-hydrocarbon lubricant. It is another object of the present invention to provide a novel method for the preparation of a lubricant useful at low temperatures. It is still another object of this invention to provide a novel method for the preparation of a lubricant possessing inherent extreme pressure properties. Other objects will become evident from the following disclosure.

Now, in accordance with this invention, it has been found that the lubricant adducts of unsaturated organic compounds, especially those containing olefinic linkages, with such sulfur-bearing substances as hydrogen sulfide or mercaptans, may be produced in yields substantially

higher than by previously known methods, by using a peroxide to catalyze the formation of the adduct.

The unsaturated organic compounds from which the lubricant may be prepared possess at least one unsaturated linkage between two aliphatic carbon atoms regardless of the character of the compound embracing such a linkage. The unsaturated hydrocarbons, such as the olefins, which term is intended to include poly-olefins and olefin polymers, are particularly contemplated. Examples of unsaturated hydrocarbons are: ethylene, propylene, 1-butene, 2-butene, isobutylene, the amylanes, 1-hexene, 2-hexene, 4-methyl-1-pentene, 4-methyl-2-pentene, 4,4-dimethyl-1-pentene, 1-octene, 1-decene, 1-cetene, styrene, cyclohexene, 3-methyl-cyclohexane, 1,4-diphenyl-2-butene, 1,3-butadiene, 1,3-pentadiene, 1,4-pentadiene, 1,4-hexadiene, 1,5-hexadiene, acetylene, methyl vinyl acetylene, octyl-acetylene, phenyl acetylene, and their homologs and analogs.

The unsaturated hydrocarbons of the above-defined class may also have one or more of their hydrogen atoms substituted by suitable organic and/or inorganic substituents, which may include substituents such as alkoxy, alkenoxy, aryloxy, alkaryloxy, aralkyloxy, alkylimido, etc. As examples, reference may be made to methylacrylate, methyl-methacrylate, divinyl ether, diallyl ether, dimethylallyl ether, allyl alcohol, diallyl sulfide, diallyl disulfide, and the like.

The lubricants prepared according to the present invention are especially versatile if the unsaturated compound has terminal aliphatic unsaturated linkages. The unsaturated ethers such as diallyl ether and divinyl ether meet this latter requirement and are a preferred class of substances useful in the preparation of the lubricants of the present invention. One group of such unsaturated ethers comprises the aliphatic oxyethers in which only one of the aliphatic radicals attached to the ether oxygen atom contains an unsaturated linkage. Examples of such ethers are ethyl vinyl ether, ethyl propenyl ether, methyl isopropenyl ether, ethyl isopropenyl ether, methyl allyl ether, ethyl allyl ether, n-propyl allyl ether, isopropyl allyl ether, 4-ethoxybutene-1, 6-ethoxy-hexene-1, gamma-ethoxy-alpha-butylene, methyl propargyl ether, ethyl propargyl ether, etc., and their homologs and analogs. The above unsaturated ethers and their homologs may be substituted by straight-chain, cyclic and/or heterocyclic radicals, as well as by 55 halogens.

Another group of suitable unsaturated ethers which may be employed as a starting material in preparing the lubricants of the present invention comprises the aliphatic thioethers in which only one of the radicals attached to the thioether sulfur atom contains an unsaturated linkage. Examples of this group are ethyl vinyl sulfide, ethyl isopropenyl sulfide, and the like.

While suitable lubricants may be prepared from the above types of unsaturated ethers, it is preferred that both radicals attached to the ether oxygen or thioether sulfur group contain unsaturated (preferably olefinic) linkages, since the adducts formed therefrom usually contain a relatively large fraction having superior lubricating properties. The following are illustrative examples of such poly-unsaturated ethers: divinyl ether, diisopropenyl ether, diallyl ether, dicrotyl ether, dimethallyl ether, di(alpha-methyl-allyl) ether, (butene-1-yl-3) (butene-2-yl-4) ether, dihexenyl ethers, allyl(2-methyl-pentene-1-yl-2) ether, allyl linallyl ether, etc., as well as the halogenated derivatives of the type of hexachlorodivinyl ethers, etc. The corresponding thioethers in which each radical attached to the sulfur atom contains an unsaturated linkage between two carbon atoms include divinyl sulfide, di(beta-chlorovinyl) thioether, diallyl sulfide, dicrotyl sulfide, dimethallyl sulfide, dihexenyl sulfides, and the like, and their homologs and analogs.

The ethers employed as the starting material for the preparation of the present lubricants may also contain more than one ether oxygen atom and/or thioether sulfur atom, this group of unsaturated ethers being represented by compounds of the type of 1,2-bis(vinyloxy) ethane, 1,3-bis(vinyloxy) propane, 1,2-bis(allyloxy) ethane, and the like, as well as by the unsaturated disulfides, such as divinyl disulfide.

At times, especially for extreme pressure lubricant purposes, it is highly desirable that a halogen-containing lubricant be employed. For this purpose, in accordance with the present invention, lubricants may be prepared from adducts, involving a halogenated unsaturated organic compound. Such halogenated unsaturated compounds may contain one or more olefinic linkages, preferably of olefinic character. These compounds may contain one or more halogen (i.e. chlorine, bromine, iodine and/or fluorine) atoms which may be attached to saturated or unsaturated carbon atoms of the compound.

Examples of such halogenated hydrocarbons are: vinyl halides, allyl halides, 2-halo-propylene, crotyl halides, isocrotyl halides, 4-halo-butene-1-methallyl halides, 2-halo-butene-2, monohalogenated acetylenes, propargyl halides, 1,1-dihaloethylenes, trihalo-ethylenes, 2-halo-pentene-1, 3-halo-cyclohexane, 2 - halo-1,4 - diphenyl - butene-2,3-halo-pentadiene-1,4, and their homologs. The above class of halogenated compounds may be further substituted in the nucleus and/or in the substituents in various degrees by straight-chain, branched chain, carbocyclic, and/or heterocyclic radicals, and by such substituents as alkoxy, alkenoxy, aryloxy, alkylimido, and the like. Also, the organic compounds of the above class may contain two or more halogen atoms which may be attached to saturated and/or unsaturated carbon atoms.

As stated hereinbefore, the adducts from which the present lubricants are derived are formed by reaction of one or more of the above unsaturated organic compounds with hydrogen sulfide or a mercaptan in the presence of an organic peroxide,

Any sufficiently stable aliphatic mercaptan is suitable as a reactant for the formation of such adducts. A suitable aliphatic mercaptan may contain one or more sulphydryl groups or radicals, preferably di- or polymercaptans. In the majority of cases it is preferable to employ mercaptans of primary, secondary or tertiary character, particularly those contained or derived from petroleum or petroleum products. The methyl, ethyl, butyl, amyl, hexyl, heptyl, octyl and the like mercaptans as well as their homologs, analogs and substitution products, may be employed with excellent results.

10 The formation of adducts of unsaturated organic compounds and hydrogen sulfide or mercaptans in the presence of peroxides proceeds according to the mechanism in which the sulfur of the mercapto or sulphydryl group attaches predominately to the unsaturated carbon atom holding the most hydrogen atoms.

15 The formation of adducts of unsaturated organic compounds and hydrogen sulfide or mercaptans in the presence of peroxides proceeds according to the mechanism in which the sulfur of the mercapto or sulphydryl group attaches predominately to the unsaturated carbon atom holding the most hydrogen atoms.

20 This type of addition is termed "abnormal," since it takes place contrary to the course suggested by the Markownikoff rule. The "abnormal" addition previously has been catalyzed by actinic radiations. This reaction is seriously limited in many cases by non-chain initiating absorption of actinic radiation. The "abnormal" addition is in accordance with the rule proposed by Posner (Berichte 38,646 (1904)). Now it has

25 been discovered, in accordance with the present invention that organic peroxides are an outstanding group of sensitizers for the purpose of producing lubricants, under proper conditions, since an exceptionally large proportion of the product so derived has lubricating properties.

30 The reaction is carried out by heating the unsaturated organic compound and hydrogen sulfide or a mercaptan in the presence of an organic peroxide, preferably in a closed vessel.

35 The peroxides preferably are organic peroxides such as the alkyl hydroperoxides, dialkyl peroxides, and alkylperoxy hydrocarbon derivatives.

40 The alkyl hydroperoxides form a preferred group of catalysts, and of these the tertiary-alkyl hydroperoxides are the most active. These include tertiary-butyl hydroperoxide, tertiary-amyl hydroperoxide, tertiary-hexyl hydroperoxide, etc. An especially preferred class of peroxides are the dialkyl peroxides, and of these, the di-tertiary-alkyl peroxides are the most satisfactory. This

45 group is exemplified by di-tertiary-butyl peroxide, di-tertiaryamyl-peroxide, di-tert-hexyl peroxide, etc.

50 Other peroxides which act as catalysts include alkyl peroxy alkanes, such as 2,2-bis(tertiary-butylperoxy) butane, as well as peroxides such as benzoyl peroxide, acetyl peroxide, benzoyl acetyl peroxide, and lauroyl peroxide, and hydroxyalkyl peroxides, such as hydroxy methyl tertiary butyl peroxide.

55 The peroxide catalyst may be used in a wide range of concentration, but preferably is present in amounts from about 1 mol per cent to about 10 mol per cent, based on the total mols of reactants present. Optimum results are obtained when the catalyst concentration is from about 2 to about 5 mol per cent.

60 The ratio of unsaturate to hydrogen sulfide or mercaptan may vary within relatively wide limits, but preferably is between 0.5 and 2 mols unsaturate to 1 mol hydrogen sulfide or mercaptan.

65 The temperature at which the reaction is conducted will depend to a certain extent on the concentration, activity and stability of the peroxide catalyst. If temperatures above 150° C. are used

when the catalyst concentration is as high as 10 mol per cent, the reaction may become violent even to the point of explosion. However, if an active peroxide is present, even in amounts as low as about one mole per cent, the reaction will proceed at a satisfactory rate at temperatures as low as about 40° C. It is preferable, from an economic and control standpoint, and when using about 2½ mol per cent of a catalyst of the activity of di-tertiary-butyl peroxide, to maintain the temperature within the range from about 100° C. to about 140° C.

The time for which the adduct reaction is allowed to proceed will vary with the activity of the catalyst and the temperature being employed. Usually the reaction will be completed when the other conditions are as stated hereinbefore, in from about 1 to about 48 hours, and close control of the reaction is obtained when conditions are such that the reaction time is from about 2 to about 10 hours. 15 20

Diluents may or may not be used, as desired. While they are not essential, their use at times may be preferable in order to reduce the viscosity of the reaction mixture, to act as a mutual solvent for the reactants and catalyst, or to reduce the concentration of the reactants, thus allowing close control of the course of the reaction. Preferably, the diluent is substantially inert with respect to the reactants or catalysts. Saturated hydrocarbons or chlorinated saturated hydrocarbons are useful for this purpose. However, reactive diluents may be used for the purpose of initiating or terminating polymer chains, so as to give adducts having modified properties as more particularly pointed out hereinafter.

The reaction proceeds at its optimum rate when retardants such as hydroquinone, piperidine, and certain metal salts are absent. Upon completion of the formation of the adduct, the product is further treated to eliminate that fraction of the product which is too volatile, or otherwise unsuitable, for use as a lubricant. This treatment may vary with the product and the type of lubricant desired, but usually comprises selective solvent extraction for the removal of catalyst and undesirable fractions, or partial distillation, usually under diminished pressure, or a combination of these two steps.

An essential feature of the present invention is the substantially complete removal of the volatile components of the adduct. Since the adduct reaction usually results in the formation of a mixture of products of continuously varying molecular weight, this relatively volatile fraction will vary in amount, dependent upon the conditions under which the adduct is formed. The sensitizer employed and its amount will have a great effect upon the proportion of relatively volatile components in the product. 50 55

When peroxides are used to catalyze the formation of the adduct, it has been found, in accordance with this invention, that the proportion of fractions having lubricating properties is unusually high, as compared with the yield obtained when other catalysts are employed. 65

The fraction of relatively volatile constituents removed will depend upon the lubricating purpose for which the remainder will be employed. If no fraction is removed the composite adduct is generally useless as a lubricant since the lighter fractions will inevitably volatilize during a lubrication operation to a greater or less degree, dependent upon the conditions to which the adduct is subjected. However, for general 70 75

5 lubricating purposes, the fraction volatilizing below about 100° C. at 0.2 cm. mercury pressure is preferably removed, and generally, that fraction volatilizing below about 160° C. at 0.2 cm. mercury pressure is removed in order to obtain a lubricant having optimum properties.

The lubricant so obtained may be further treated in order to improve color, alter terminal groups, etc., if desired.

10. The adducts formed by the above reaction may contain sulfhydryl or mercapto groups attached to one of the carbon atoms initially having an unsaturated linkage.

When ethers or thioethers having unsaturated linkages in both radicals attached to the ether oxygen or thioether sulfur atom are treated with hydrogen sulfide or a mercaptan as described hereinbefore, the adducts are polymeric compounds having units of the general configuration



25 wherein X is either sulfur or oxygen (dependent upon whether an ether or a thioether was used) and each R is an organic radical, preferably a saturated hydrocarbon radical, of from 1 to 20 carbons.

When the adduct is formed from hydrogen sulfide and an oxyether having unsaturated linkages in both radicals attached to the ether oxygen atom, the polymer has the general formula



35 wherein  $R_2$  and  $R_3$  represent like or different substituted or unsubstituted hydrocarbon radicals,  $m$  is an integer,  $R_1$  represents the hydrogen atom or radicals such as  $-\text{CH}_2-$ ,  $R_5$  represents the sulphydryl radical or radicals such as  $-\text{S}-\text{CH}_2-$ ,  $R_7$  represents the hydrogen atom or radicals such as  $-\text{CH}_2-\text{R}_6-\text{O}-\text{R}_8-\text{CH}_2$ , wherein  $R_5$  through  $R_8$  represent like or different substituted or unsubstituted hydrocarbon radicals. An outstanding member of this group is the adduct of diallyl ether and hydrogen sulfide.

When an unsaturated thioether is treated with hydrogen sulfide, the polymer corresponds to that above, except that the oxygen atoms are all replaced by sulfur atoms, thus giving a polymer having a high sulfur content, especially useful for extreme pressure lubrication. An outstanding member of this group is the adduct of diallyl sulfide and hydrogen sulfide.

The adducts formed according to the method of the present invention are particularly useful in the preparation of lubricants, since the use of peroxide catalysts enables the production of a large fraction having lubricating properties. The adducts so formed are stable to oxidation and may be used in the preparation of lubricants.

and respond well to certain anti-oxidants, such as 1,2-dihydroxybenzene. They have low pour points (usually lower than -30° F.) and exhibit exceptional extreme pressure characteristics. They may be used by themselves as lubricants, or may be added to other lubricant bases, such as mineral oils, polymeric alkylene oxides or glycols, high molecular weight esters, etc., in order to create extreme pressure lubricant compositions. The subject adducts may be combined with other materials, such as gelling agents to produce greases; organic acids to produce anti-corrosion compositions, etc. They are especially suitable for use in cutting oil compositions.

The following examples illustrate the method of the present invention, and the use of the adducts so prepared.

**EXAMPLE I.—PEROXIDE CATALYZED ADDUCT OF H<sub>2</sub>S AND DIALLYL ETHER**

Equimolecular amounts of hydrogen sulfide and diallyl ether, together with 5 mol percent di-tertiary-butyl peroxide were heated in an autoclave at 100° C. for 30 hours. Following adduct formation, the more volatile fractions were removed by fractional distillation at sub-atmospheric pressure. The fraction of the product boiling above 240° C. at 0.2 cm. mercury pressure (70% of the charge) had the following properties:

|                                   |      |    |
|-----------------------------------|------|----|
| Viscosity centistokes at 100° F.  | 77.0 | 10 |
| Viscosity, centistokes at 210° F. | 13.0 | 15 |
| Viscosity index                   | 143  |    |
| S. A. E. grade                    | 30   |    |
| Pour point, °F.                   | -60  |    |

**EXAMPLE II.—PEROXIDE CATALYZED ADDUCT OF H<sub>2</sub>S AND DIALLYL ETHER**

Adducts were prepared as described in Example I, using several different peroxides, heating for 20 hours at 65° C. The yields of product boiling above 160° C. at 0.2 cm. mercury pressure are given in Table I, below.

Table I

| Peroxide                                  | Per cent Yield of Lubricant Fraction | 30 |
|-------------------------------------------|--------------------------------------|----|
| 2,2-bis(tertiary-butylperoxy)butane       | 30                                   |    |
| tertiary-Butyl hydroperoxide <sup>1</sup> | 67                                   |    |
| Lauroyl peroxide                          | 25                                   |    |
| Benzoyl peroxide                          | 20                                   |    |

<sup>1</sup> Reaction mixture heated 30 hours at 100° C.

**EXAMPLE III.—LAUSON ENGINE TEST ON H<sub>2</sub>S-DIALLYL ETHER ADDUCT**

The adduct prepared as described in Example I was tested as a lubricant in a standard Lauson engine, operated at a jacket temperature of 100° F. for 40 hours. The following characteristics were observed:

|                                        |        |    |
|----------------------------------------|--------|----|
| Bearing weight loss, mgs. per sq. cm.  | 7.3    | 45 |
| Oil consumption                        | Normal |    |
| Sludge deposits                        | None   |    |
| Ring belt deposits                     | Medium |    |
| Wear                                   | Normal |    |
| Approximate S. A. E. grade             | 20     |    |
| Percent viscosity increase during test | 42     |    |

**EXAMPLE IV.—WEAR TEST—H<sub>2</sub>S ADDUCTS OF DIALLYL ETHER**

Two adducts of hydrogen sulfide and diallyl ether, were tested for wear characteristics in the four-ball wear apparatus described by Boelage in "Engineering" (June 14, 1933). Results of the test are given in Table 2 below.

Table 2

|                                                           |       |       |            |
|-----------------------------------------------------------|-------|-------|------------|
| Molecular weight of adduct                                | 584   | 476   | 60         |
| Pour point, °C.                                           | -43   | -55   |            |
| At 30° C., 1200 R. P. M., 15 kg. load:                    |       |       |            |
| Average diameter of wear sec., mm.                        | 0.23  | 0.26  | 70         |
| Coefficient of friction after 5 seconds                   | 0.062 | 0.066 |            |
| Coefficient of friction average of 30, 40, 50 and 60 sec. | 0.059 | 0.068 | 75 tained. |

|                                                           |       |       |  |
|-----------------------------------------------------------|-------|-------|--|
| At 80° C., 1200 R. P. M., 15 kg. load:                    |       |       |  |
| Average diameter of wear scar, mm.                        | 0.25  | 0.26  |  |
| Coefficient of friction after 5 seconds                   | 0.056 | 0.066 |  |
| Coefficient of friction average of 30, 40, 50 and 60 sec. | 0.054 | 0.063 |  |
| At 130° C., 1200 R. P. M., 15 kg. load:                   |       |       |  |
| Average diameter of wear scar, mm.                        | 0.26  | 0.27  |  |
| Coefficient of friction after 5 seconds                   | 0.045 | 0.061 |  |
| Coefficient of friction average of 30, 40, 50 and 60 sec. | 0.043 | 0.058 |  |
| At 30° C., 700 R. P. M., 7 kg. load, two hour test:       |       |       |  |
| Scar diameter, mm.                                        | 0.40  | —     |  |
| Average coefficient of friction during the 2 hr. test     | 0.061 | —     |  |
| At 80° C., 700 R. P. M., 7 kg. load, 2 hour test:         |       |       |  |
| Scar diameter, mm.                                        | 0.48  | —     |  |
| Average coefficient of friction during the 2 hr. test     | 0.058 | —     |  |
| At 130° C., 700 R. P. M., 7 kg. load, 2 hour test:        |       |       |  |
| Scar diameter, mm.                                        | 0.33  | 0.38  |  |
| Average coefficient of friction during 2 hr. test         | 0.073 | 0.080 |  |

**EXAMPLE V.—THERMAL STABILITY OF THE H<sub>2</sub>S-DIALLYL ETHER ADDUCT**

The adduct prepared as described in Example I was heated for 24 hours at 150° C. in a carbon dioxide atmosphere in order to determine what changes occur in its properties in the absence of oxidizing influences. Table 3 presents the data obtained:

Table 3

|                                  |             |  |  |
|----------------------------------|-------------|--|--|
| Before testing:                  |             |  |  |
| Viscosity—centistokes at 100° F. | 40.7        |  |  |
| Viscosity—centistokes at 210° F. | 7.85        |  |  |
| Viscosity index                  | 149         |  |  |
| Color                            | Yellow      |  |  |
| After testing:                   |             |  |  |
| Viscosity—centistokes at 100° F. | 42.1        |  |  |
| Viscosity—centistokes at 210° F. | 8.09        |  |  |
| Viscosity index                  | 149         |  |  |
| Color                            | Dark yellow |  |  |

**EXAMPLE VI.—OXIDATION STABILITY OF H<sub>2</sub>S-DIALLYL ETHER ADDUCT**

Seventy-five grams of the adduct of diallyl ether and hydrogen sulfide, prepared as described in Example I were heated at 140° C. in the presence of 1 sq. cm. copper per gram oil under an initial oxygen pressure of 50 p. s. i. It required 11.5 hours heating under these conditions for the oxygen pressure to drop 10 p. s. i. and 26 hours for the pressure to drop 20 p. s. i.

**EXAMPLE VII.—EXTREME PRESSURE LUBRICATING PROPERTIES OF THE H<sub>2</sub>S-DIALLYL ETHER ADDUCT**

The adduct prepared as described in Example I was tested under loads simulating extreme pressure lubricating conditions, using the four-ball machine described by Boelage in "Engineering" (June 14, 1933). Table 4 presents the data obtained.

**9**  
*Table 4*

| Load (kg.) | Scar Diameter |
|------------|---------------|
| 40         | 0.36          |
| 60         | 0.42          |
| 80         | 0.46          |
| 100        | 0.86          |
| 200        | 1.52          |
| 300        | 2.51          |
| 400        | 3.24          |
| 500        | 3.37          |
| 700        | 3.61          |

We claim as our invention:

1. The process which comprises heating hydrogen sulfide and diallyl ether in the presence of a minor amount of di-tertiary-butyl peroxide at a temperature from 40° to 150° C. for a period between one and 48 hours and removing from the mixture of polymeric adducts so formed the fraction volatilizing below 160° C. at 1 cm. mercury pressure.

2. The process which comprises heating hydrogen sulfide and diallyl ether in the presence of a dialkyl peroxide at a temperature between 40° and 150° C., and removing from the mixture of linear polymeric adducts so formed the fraction volatilizing below 160° C. at 1 cm. mercury pressure.

3. The process which comprises heating hydrogen sulfide and a dialkenyl ether in the presence of a catalyst of the group consisting of dialkyl peroxides and alkyl hydroperoxides, and removing from the mixture of linear polymeric adducts so formed the fraction volatilizing below 160° C. at 1 cm. mercury pressure.

4. The process which comprises heating a sulfur compound having the general formula

**R—S—R**

wherein both R's are of the group consisting of hydrogen atoms and alkyl radicals, at least one R being a hydrogen atom, with a dialkenyl ether, in the presence of a minor amount of a catalyst of the group consisting of dialkylperoxides and alkyl hydroperoxides, whereby a mixture of polymeric linear adducts of the reactants is formed, and subsequently removing from said mixture the fraction which volatilizes below 160° C. at 1 cm. mercury pressure.

5. The process which comprises heating an alkyl mercaptan with a dialkenyl ether in the presence of a minor amount of a catalyst of the group consisting of dialkyl peroxides and alkyl hydroperoxides, whereby a mixture of polymeric linear adducts of the reactants is formed and subsequently removing from said mixture the fraction which volatilizes below 160° C. at 1 cm. mercury pressure.

6. The process which comprises heating a sulfur compound having the general formula

**R—S—R**

wherein both R's are of the group consisting of hydrogen atoms and alkyl radicals, at least one

**10**

R being a hydrogen atom, with a dialkenyl ether in the presence of a minor amount of a dialkyl peroxide, whereby a mixture of polymeric linear adducts of the reactants is formed and subsequently removing from said mixture the fraction which volatilizes below 160° C. at 1 cm. mercury pressure.

5 7. The process which comprises heating a sulfur compound having the general formula

10

**R—S—R**

wherein both R's are of the group consisting of hydrogen atoms and alkyl radicals, at least one R being a hydrogen atom, with a dialkenyl ether in the presence of a minor amount of an alkyl peroxide, whereby a mixture of polymeric linear adducts of the reactants is formed and subsequently removing from said mixture the fraction which volatilizes below 160° C. at 1 cm. mercury pressure.

20

8. The process which comprises heating hydrogen sulfide having a dialkenyl ether in the presence of a dialkyl peroxide catalyst and removing from the mixture of linear polymeric adducts so formed, the fraction volatilizing below 160° C. at 1 cm. mercury pressure.

25

9. The process which comprises heating hydrogen sulfide having a dialkenyl ether in the presence of an alkyl hydroperoxide catalyst and removing from the mixture of linear polymeric adducts so formed, the fraction volatilizing below 160° C. at 1 cm. mercury pressure.

30

10. The process which comprises heating hydrogen sulfide and divinyl ether in the presence of a catalyst of the group consisting of dialkyl peroxides and alkyl hydroperoxides and removing from the mixture of linear polymeric adducts so formed, the fraction volatilizing below 160° C. at 1 cm. mercury pressure.

35

11. The following references are of record in the

file of this patent:

**UNITED STATES PATENTS**

| Number       | Name               | Date          |
|--------------|--------------------|---------------|
| 50 2,197,781 | Badertscher et al. | Apr. 23, 1940 |
| 2,319,183    | Badertscher et al. | May 11, 1943  |
| 2,352,435    | Hoeffelman et al.  | June 27, 1944 |
| 2,373,343    | Rummelsburg        | Apr. 10, 1945 |
| 2,392,295    | Rust et al.        | Jan. 1, 1946  |

**OTHER REFERENCES**

- Jour. of A. C. S. (1938) 60: 2452 to 2455.  
 Chem. Rev. (1942) 27: 383 to 394.  
 Vaughn et al.: Jour. Organic Chem., vol. 7, pages 472-6 (1942).  
 Jones et al.: Jour. Am. Chem. Soc., vol. 60, page 2452 (1938).  
 Kharasch et al.: Chemistry and Industry, vol. 57, page 752 (1938).